

## UNITED STATES PATENT OFFICE

2,403,927

## IMPROVERS FOR PHOTOGRAPHIC EMULSIONS

John David Kendall, Douglas James Fry, and James Douglas Brooks, Ilford, England, assignors to Ilford Limited, Ilford, Essex, England, a British company

No Drawing. Application November 12, 1943, Serial No. 510,040. In Great Britain December 3, 1942

21 Claims. (Cl. 95—6)

1

This invention relates to compounds which serve as improvers for photographic silver halide emulsions and particularly to compounds which, when added to the emulsion, or to the developer used in processing the emulsion, or otherwise applied to the emulsion before development, improve the quality of the developed photographic image obtained.

On exposure and development of a normal photographic film, plate or paper bearing a silver halide photographic emulsion there is produced, in addition to the silver image, a general deposit of metallic silver, the distribution and density of which bears no direct relation to the variations in luminosity of the subject. This overall deposit is referred to as "chemical fog" or "development fog." Its effect is to increase the general density of the negative obtained and to depress the contrast of the image in the least exposed parts. In general the fog density produced is greater in the case of high speed emulsions than in slow emulsions, and it is invariably greater the more complete the development, e. g. the higher the temperature of development, and when vigorous developers are used.

Moreover, the degree to which an emulsion produces fog on development usually increases with the age of the emulsion, so that photographic emulsions which have been kept a long time, especially in warm or humid conditions, and emulsions which have been kept a long time in the molten condition, may produce images associated with a heavy fog density. Many compounds have been suggested in the past for use as additions to emulsions or to developers which tend to reduce the formation of fog, but almost all of them, if reasonably effective as anti-fogging agents, have caused a serious reduction in the speed of the photographic emulsion.

Further, in the production of photographic images in silver halide photographic emulsions, and particularly in the case of emulsions consisting primarily of silver chloride, the maximum image density obtainable is not always so great as may be desired. Moreover, the common practice of hot-glazing photographic prints tends to affect adversely the image colour, giving a poor quality black known as the "bronzing" effect, and also reduces the effective maximum density obtainable in the image.

It has now been discovered, and this forms the basis of the present invention, that the treatment of a photographic silver halide emulsion with a small quantity of a 5-mercaptop-tetrazole, of the general tautomeric formulae:



2

where R is a hydrogen atom or a hydrocarbon substituent group (which itself may be substituted or unsubstituted), at a stage not later than the development of the emulsion, has a considerable improving effect on the quality of the developed photographic image in respect of the characteristics referred to above.

The compounds are preferably included in the emulsion during its manufacture, or in the developer used, but any other method of bringing the compounds into operative contact with the emulsion may be used, for example the compounds may be included in subcoat, supercoat or backing layers which are, or become, in contact with the emulsion, or they may be included in the wrapping materials used, or they may be applied to the emulsion in solution before the emulsion is developed.

The compounds of this invention are not equally effective in all respects, and it has been found that whilst all of them serve to reduce development fog to some extent and also serve to cause an effective increase in maximum image density, especially after hot glazing, nevertheless,

some compounds of the series are better for one purpose than for the other. Thus, for example, where the primary object is to stabilise the emulsion, or to reduce the fog density of the developed image, those compounds of the above general formulae in which R is an aryl, substituted aryl, aralkyl or cycloalkyl group are preferred. The compounds in which R is a hydrogen atom or an alkyl group, though effective, are generally less satisfactory from this standpoint. The aryl, substituted-aryl, aralkyl and cycloalkyl compounds are effective anti-fogging agents, however brought into operative contact with the emulsion, but they are preferred for use in developers or in the emulsions. The compound 1-phenyl-5-mercaptop-tetrazole is typical of this class, and it is found to preserve high speed photographic emulsions against excessive fog over long periods of time and also to enable development to be effected with vigorous developers or at high temperatures. Thus, these compounds are of particular value as emulsion or developer additions in cases where the emulsions or developers are to be used in tropical

conditions or, in the case of emulsions, where the emulsions are to be kept for a long time in the molten condition. These compounds further present the advantage that their use in concentrations sufficient to cause a useful fog reduction does not seriously reduce the effective speed of the emulsions in which they are incorporated, or to which they are applied in developer solution, and in some cases the compounds actually increase the effective speed.

All the compounds, whatever the nature of the 1-substituent (if any), have a valuable effect in increasing the maximum density obtainable in the developed image. They not only tend to increase the maximum image density in the case of normally "cold-dried" images, but also lead to a marked increase in the maximum image density where the images are hot-glazed. Furthermore, the compounds substantially prevent the bronzing effect which, as stated above, has been a common disadvantage in the hot-glazing process.

Improvement in maximum image density is best obtained where the compounds are included in the emulsion or in the developer or both, and it will be appreciated that by using a compound of the type where the group R is an aryl, substituted aryl, aralkyl or cycloalkyl group, an increase in maximum image density, a decrease in bronzing on hot-glazing and a decrease in the fog level can be simultaneously obtained with especially good effect.

The compounds of the invention may be prepared by condensing an azide such as sodium azide with a mustard oil (i.e. a compound of the structure R.NCS where R is a hydrocarbon group) as described by Stollé and Strittmatter in the *Journal für Praktische Chemie*, volume 133, pages 60-64, and by Stollé and Fr. Henke-Stark in the same journal, volume 124, pages 261-300. An alternative method for production of the aryl-substituted compounds is by treatment of an aryl thiosemicarbazide with nitrous acid, as described by Freund and Hempel in *Berichte der Deutschen Chemischen Gesellschaft*, volume 28, at page 77.

As indicated above, the group R in the tautomeric general formulae may be a hydrogen atom or a hydrocarbon group. Examples of the latter are alkyl groups, e.g. methyl, ethyl and higher alkyl groups, and unsaturated groups of this type, e.g. allyl; aryl groups, e.g. phenyl and naphthyl; aralkyl groups, e.g. benzyl; and cycloalkyl groups, e.g. cyclohexyl. Such groups may themselves be substituted, for example, by halogen atoms or amino groups.

The quantity of the compound employed will depend on the manner in which it is brought into operative contact with the emulsion, but as a general indication it may be stated that for incorporation in an emulsion, 1 to 5 or up to 20 cc. of a 1:1,000 solution of the compound per litre of emulsion is suitable, whilst for incorporation in a developer, the optimum quantity may vary from 1 part of the compound in 3,000 to 100,000 parts of the developer solution according to the particular compound used. The addition of the compound to an emulsion is preferably effected after the digestion of the emulsion, as a final addition before coating.

The following examples illustrate the invention:

(a) *Preparation of 1-phenyl-5-mercapto tetrazole.*—5 gms. of 4-phenyl-thio-semicarbazide, 3.5 ccs. of concentrated hydrochloric acid, and 100 ccs. of water were mixed together and cooled in ice. The mixture was vigorously stirred and there was slowly added, in portions, 2.1 gms. of solid sodium nitrite. A white precipitate formed and the stirring was continued for 15 minutes after all the sodium nitrite had been added. The precipitate was then filtered off, washed with water and then immediately dissolved in 25 ccs. of 10% aqueous sodium carbonate solution by boiling. The hot solution was filtered and the filtrate allowed to cool. The filtrate was then

acidified with hydrochloric acid, whereupon the desired compound was precipitated. It was filtered off, washed with water and re-crystallised from aqueous alcohol solution. It has a melting point of 155° C. with decomposition.

(b) *Use of 1-phenyl-5-mercapto-tetrazole in an emulsion.*—A standard gelatino silver iodobromide emulsion having a silver content of 28.5 gms. per litre (calculated as metallic silver) was prepared. One portion of the emulsion was tested as a control, and to other portions quantities of 1-phenyl-5-mercapto tetrazole were added. The fog values and speed values of the separate portions of the emulsion were determined immediately after coating, and again after being kept for several days in a moist warm atmosphere. The original relative speed of the control emulsion was taken as 100. The results obtained are set out in the following Table I.

Table I

| Quantity of compound added per litre of emulsion | Immediately after coating |             | After keeping  |             |
|--------------------------------------------------|---------------------------|-------------|----------------|-------------|
|                                                  | Relative speed            | Fog density | Relative speed | Fog density |
| 0                                                | 100                       | 0.05        | 60             | 0.53        |
| 2 ccs. of 1:1,000 solution                       | 92                        | 0.05        | 72             | 0.23        |
| 4 ccs. of 1:1,000 solution                       | 88                        | 0.04        | 80             | 0.10        |

It will be observed that the addition of 4 ccs. of a 1 in 1,000 solution of the compound per litre of emulsion effects a very considerable reduction in the fog value, especially after keeping, and stabilises the speed of the emulsion to a value not seriously below that of the untreated emulsion.

(c) *Use of 1-phenyl-5-mercapto tetrazole in a developer.*—A high speed panchromatic film was developed for 1 minute at 100° F. in a standard high temperature developing solution. Three tests were made, one with the normal developing solution to serve as a control, and two others with different added quantities of 1-phenyl-5-mercapto tetrazole. The speed and fog values were determined and gave the results set out in the following Table II. The initial relative speed of the control emulsion was again taken as 100.

Table II

| Quantity of compound added to developer | Relative speed | Fog value |
|-----------------------------------------|----------------|-----------|
| 0                                       | 100            | 0.86      |
| 1 part in 30,000 of developer           | 200            | 0.50      |
| 1 part in 10,000 of developer           | 140            | 0.10      |

Example II

This example illustrates the results obtainable with variously substituted 5-mercapto tetrazoles included in a photographic silver iodobromide emulsion.

The results obtained on a series of tests are set out in Table III where in each line there is given the nature of the 1-substituent, the quantity of compound added to the emulsion, the fog value of a control sample of the emulsion not containing the compound, and lastly the fog value of a test sample containing the stated quantity of the stated compound. The variation in the figures for the control tests is due to the fact that separate controls were effected for each case, using

different batches of emulsion and varying to some extent the emulsion-making conditions.

Table III

| 1-substituent          | Addition in<br>ccs. 1:1,000<br>solution per<br>litre of<br>emulsion | Fog values after<br>keeping |                |
|------------------------|---------------------------------------------------------------------|-----------------------------|----------------|
|                        |                                                                     | Control                     | Test<br>sample |
| None                   | 2.5                                                                 | 0.34                        | 0.22           |
| $\alpha$ -naphthyl     | 5.4                                                                 | 0.31                        | 0.13           |
| p-diethyl-amino-phenyl | 6.0                                                                 | 0.66                        | 0.24           |
| o-methoxy phenyl       | 4.6                                                                 | 0.50                        | 0.15           |
| p-chlor-phenyl         | 6.2                                                                 | 0.32                        | 0.12           |
| Benzyl                 | 5.6                                                                 | 0.60                        | 0.23           |
| Cyclohexyl             | 4.4                                                                 | 0.66                        | 0.16           |
| Methyl                 | 2.8                                                                 | 0.45                        | 0.28           |
| Ethyl                  | 3.2                                                                 | 0.34                        | 0.24           |

It will be seen that in every case the compounds are effective in reducing the fog density of the developed images, and this table also illustrates the statement previously made that the substituted aryl, aralkyl and cyclo-alkyl compounds are generally more effective than the alkyl and unsubstituted compounds of the series, though quite useful improvements are obtained with these latter compounds.

*Example III.—The use of 1-methyl 5-mercaptop-tetrazole in a developer*

Exposed samples of a photographic printing paper of the so-called "contact" type (essentially a silver chloride emulsion) were developed for one minute at 65° F. in a standard metol hydroquinone developer. Two tests are made, one with the normal developing solution and one with a developer containing an addition of 1 part in 10,000 of 1-methyl-5-mercaptop-tetrazole. The test samples were processed normally and finally glazed on a commercial hot glazing machine. The test sample developed in the absence of 1-methyl-5-mercaptop-tetrazole showed a bronzed image having a maximum reflection density of 1.55, while that developed in the presence of 1-methyl-5-mercaptop-tetrazole showed a good black image of maximum reflection density 1.95.

*Example 4.—Use of 1- $\alpha$ -naphthyl-5-mercaptop-tetrazole in a developer*

The procedure of Example 3 was followed, but four sample strips were prepared, two (test samples) being developed in a developer containing 1- $\alpha$ -naphthyl-5-mercaptop-tetrazole and two (control) strips in the same developer not containing that compound. One strip of each pair was then normally dried in air at ordinary temperatures, and the other of the pair was glazed on a commercial hot-glazing machine. The maximum reflection density values obtained in the processed images are shown in the following Table IV:

Table IV

|            | Control | Test sample |
|------------|---------|-------------|
| Air-dried  | 1.75    | 1.9         |
| Hot-glazed | 1.55    | 2.0         |

It will be noted that the presence of 1- $\alpha$ -naphthyl-5-mercaptop-tetrazole increased the maximum reflection density even in the case of normally dried prints and effected a very substantial increase in the case of prints which were hot-glazed. The hot-glazed control print showed a considerable bronzing effect which was substantially elimi-

nated in the case of the hot-glazed sample strip containing 1- $\alpha$ -naphthyl-5-mercaptop-tetrazole.

*Example 5.—Use of 1-cyclohexyl-5-mercaptop-tetrazole in developer*

5 The procedure of Example 3 was followed precisely except that the samples were of a photographic paper of the type normally used for making enlargements (i. e. consisting essentially of silver bromide). It was found that the control sample developed in the absence of 1-cyclohexyl-5-mercaptop-tetrazole showed a somewhat bronzed image having a maximum reflection density of 1.85, while the test sample developed in the presence of the said compound showed a good black image of maximum reflection density 2.0.

*Example 6.—Use of 1-phenyl-5-mercaptop-tetrazole in a supercoat*

20 A silver halide (mainly silver chloride) photographic emulsion on paper base was coated with a gelatin supercoat containing 10 ccs. of a 1% solution of 1-phenyl-5-mercaptop-tetrazole per litre of supercoat solution. A control sample made with a plain gelatin supercoat showed on development a fog density, after keeping, of 0.13, whereas the test sample processed under the same conditions showed a fog density of only 0.04. Moreover, the test sample showed a considerable reduction, compared with the control, in the degree of bronzing of the image effected by hot-glazing the prints.

25 In the following claims, the term "5-mercaptop-tetrazole" and the references to substituents in the "1-position" are to be understood in relation to the general tautomeric formulae set out above.

What we claim is:

30 1. A method of improving photographic silver halide emulsions in regard to the quality of images developed therein, which comprises treating the emulsion, at a stage not later than its development, with a small quantity of a 5-mercaptop-tetrazole having in the 1-position thereof a group taken from the class consisting of a hydrogen atom and a hydrocarbon radical.

35 2. A method of improving photographic silver halide emulsions in regard to the quality of images developed therein, which comprises including in the emulsion during its manufacture a small quantity of a 5-mercaptop-tetrazole having in the 1-position thereof a group taken from the class consisting of a hydrogen atom and a hydrocarbon radical.

40 3. A method of improving photographic silver halide emulsions in regard to the quality of images developed therein, which comprises developing said images with a developer solution which contains a small quantity of a 5-mercaptop-tetrazole having in the 1-position thereof a group taken from the class consisting of a hydrogen atom and a hydrocarbon radical.

45 4. A method of improving photographic silver halide emulsions in regard to the quality of images developed therein, which comprises including in the emulsion during its manufacture a 5-mercaptop-tetrazole containing a cyclic hydrocarbon substituent in the 1-position.

50 5. A method of improving photographic silver halide emulsions in regard to the quality of images developed therein, which comprises developing said images with a developer solution which contains a small quantity of a 5-mercaptop-tetrazole containing a cyclic hydrocarbon substituent in the 1-position.

55 6. A method of improving photographic silver halide emulsions in regard to the quality of

images developed therein, which comprises treating the emulsion, at a stage not later than its development, with a 5-mercaptop-tetrazole containing an aryl substituent in the 1-position.

7. A method of improving photographic silver halide emulsions in regard to the quality of images developed therein, which comprises developing said images with a developer solution which contains a small quantity of a 5-mercaptop-tetrazole containing an aryl substituent in the 1-position.

8. A silver halide photographic emulsion containing a small quantity of a 5-mercaptop-tetrazole having in the 1-position thereof a group taken from the class consisting of a hydrogen atom and a hydrocarbon radical.

9. A photographic element comprising a silver halide photographic emulsion and, in contact therewith, a small quantity of a 5-mercaptop-tetrazole having in the 1-position thereof a group taken from the class consisting of a hydrogen atom and a hydrocarbon radical.

10. A silver halide photographic emulsion containing a small quantity of a 5-mercaptop-tetrazole containing a cyclic hydrocarbon substituent in the 1-position.

11. A photographic element comprising a silver halide photographic emulsion and, in contact therewith, a small quantity of a 5-mercaptop-tetrazole containing a cyclic hydrocarbon substituent in the 1-position.

12. A silver halide photographic emulsion containing a small quantity of a 5-mercaptop-tetrazole containing an aryl substituent in the 1-position.

13. A photographic element comprising a silver halide photographic emulsion and, in contact therewith, a small quantity of a 5-mercaptop-tetrazole containing an aryl substituent in the 1-position.

14. A developer for photographic silver halide emulsions containing a developing agent and a small quantity of a 5-mercaptop-tetrazole having in the 1-position thereof a group taken from the class consisting of a hydrogen atom and a hydrocarbon radical.

15. A developer for photographic silver halide emulsions containing a developing agent and a

small quantity of a 5-mercaptop-tetrazole containing a cyclic hydrocarbon substituent in the 1-position.

16. A developer for photographic silver halide emulsions containing a developing agent and a small quantity of a 5-mercaptop-tetrazole containing an aryl substituent in the 1-position.

17. A process for the production of photographic prints which comprises developing a latent image contained in a photographic silver halide emulsion on a paper support, in the presence of a small quantity of a 5-mercaptop-tetrazole having in the 1-position thereof a group taken from the class consisting of a hydrogen atom and a hydrocarbon radical.

18. A process for the production of photographic prints which comprises developing a latent image contained in a photographic silver halide emulsion on a paper support, in the presence of a small quantity of a 5-mercaptop-tetrazole containing a cyclic hydrocarbon substituent in the 1-position.

19. A process for the production of photographic prints which comprises developing a latent image contained in a photographic silver halide emulsion on a paper support, in the presence of a small quantity of a 5-mercaptop-tetrazole containing an aryl substituent in the 1-position.

20. A process for the production of photographic prints which comprises developing a latent image contained in a photographic silver halide emulsion on a paper support in the presence of a small quantity of a 5-mercaptop-tetrazole containing a hydrocarbon substituent in the 1-position and hot-glazing the paper print so obtained.

21. A silver halide photographic emulsion containing a 5-mercaptop-tetrazole having in the 1-position thereof a group taken from the class consisting of a hydrogen atom and a hydrocarbon radical in an amount corresponding to that obtained by adding 1 to 20 ccs. of a 1 to 1000 solution per liter of emulsion.

JOHN DAVID KENDALL.  
DOUGLAS JAMES FRY.  
JAMES DOUGLAS BROOKS.